

Patented Mar. 30, 1926.

1,578,405

# UNITED STATES PATENT OFFICE.

JUDSON A. DE CEW, OF MOUNT VERNON, NEW YORK.

## PROCESS OF HYDRATION IN PAPER MAKING USING FRICTION.

No Drawing.

Application filed January 20, 1925. Serial No. 3,597.

To all whom it may concern:

Be it known that I, JUDSON A. DE CEW, a subject of the King of Great Britain, and resident of Mount Vernon, in the county of 5 Westchester and State of New York, have invented certain new and useful Improvements in Processes of Hydration in Paper Making Using Friction, of which the following is a specification.

10 The following invention relates to a method for increasing the strength of paper fabric by altering the character of the surface of the fibres from which the paper is made, during the process of beating the 15 paper stock.

I have discovered that the chief factors effecting the strength of the paper fabric is the character of the surface of the fibres from which the paper is made.

20 It has been generally considered that the effect on the cellulose fibres in beating them into a condition for paper making is one of the hydration of the entire fibre itself, due to the bruising action resulting from the 25 treatment received in beaters and jordans.

It has been conceived that by chemical treatment of the fibres they may be swollen and made to absorb water, but I have discovered that the principal advantage in certain chemical treatments is the fact that certain surface phenomena occur of the nature of adsorption that will bring about a condition 30 on the surface of cellulose fibres which will make these fibres adhere to each other more firmly when formed into a sheet of paper.

The basis of my discovery is that the method of obtaining the desired result is to agitate or beat the fibres in cold water in which is dissolved a caustic alkali such as 40 caustic soda or caustic potash which will have a softening action upon the surface of the fibres while they are being rubbed against each other.

It has long been known that caustic alkali 45 will have a swelling effect upon cellulose when the solution is concentrated and cellulose may be actually dissolved by caustic at high temperatures, but for purposes of paper making by means of my process, it is 50 only desired to produce an effect upon the surface of the fibre and it is not necessary to use strong solutions which will penetrate to the interior of the cell walls or to heat the solutions.

55 My discovery applies to the treatment of any cellulose fibre for paper making, but

particularly in the preparation of sulphate cellulose which is used in the manufacture of wrapping paper. One method of operation is to carry out the beating of the fibres either in the beating engine or the jordan, or similar machine, while the water surrounding the fibres is made slightly alkaline with a solution of caustic soda or caustic potash. The result of this beating action under these conditions is that the surface of the fibres becomes slippery because the rapid movement of the fibres in the presence of the dilute caustic alkali accelerates the reactions on the surface of the fibres which produces 70 a distinctive result as compared with any method of treatment in which the fibres are not being rubbed against each other, or when the cellulose is heated with alkalis or in stronger solution than required for surface phenomena.

In fact the fibres may have a prolonged alkaline treatment without friction and then if agitated in the beater in the presence of the solutions used for sizing the fibres 80 will not make as strong a paper as when they are beaten within the alkaline solution at a consistency in which the fibres will have some friction against each other. I also find that the only alkaline solution 85 that is at all effective is a caustic alkali which has a solvent action on the surface of the fibre that is not obtained by a carbonate alkali, even of greater strength.

In the ordinary paper mill there are two 90 stages in which the fibres are made soft and pliable, one being a treatment in a beater between a revolving roll and bedplate, and the later treatment whereby the fibres pass continuously through an apparatus containing a revolving cone with knives, called jordan engines, in which the fibres are again further rubbed against each other by the moving knives. In carrying out my process, I prefer to keep the amount of water surrounding the fibres as low as possible so that the friction between the fibres will be increased by their agitation.

The proportion of alkali I find desirable 100 for practical purposes is from 2 to 8 pounds of caustic soda or potash to each 1000 pounds of fibre, this quantity being sufficient to produce the surface phenomena which takes place when the fibres are agitated in this solution.

110 The action which takes place in this process is just as beneficial to a cellulose

which has been produced by an alkaline process as one which has been produced by an acid process, and the result is not one of chemical reaction with the cellulose because after the action is completed practically all the alkali can be removed by washing if desired.

At the present time both the beating and jordaning actions are carried out in the presence of a weak solution of sulphate of alumina and as a result the fibres are astringent through surface adsorption of basic aluminum sulphate. Under these conditions with adsorbed acidity, they do not readily produce surface hydration by fibre friction, and require harder mechanical treatment.

At a concentration of fibres up to about 5%, the fibres are floating in the water surrounding them, and consequently there is little friction between them, but at a consistency of from 5% to 12% the fibres are resting against each other and when moved about the surfaces actually rub against each other. It is under this condition that sur-

face hydration can be obtained and the less water surrounding the fibres the greater the surface hydration obtainable.

Fibres that are hydrated in this manner have different physical characteristics than those that are hydrated by bruising action, and will give a paper of both pliability and strength.

In my process any treatment requiring the use of sulphate of alumina is carried out after the surface treatment of the fibres is complete.

Having thus described my invention, what I claim is:—

A method of preparing cellulose fibres for paper making, which consists in beating and jordaning the cellulose in water containing cold dilute soluble caustic alkali and then sizing the fibres by a special series of operations in which the alkalinity is neutralized.

In testimony whereof, I affix my signature.

JUDSON A. DE CEW.